

## UNITED STATES PATENT OFFICE

2,179,060

MANUFACTURE OF LUBRICATING COMPO-  
SITIONSHerschel G. Smith, Swarthmore, Pa., assignor to  
Gulf Oil Corporation, Pittsburgh, Pa., a cor-  
poration of PennsylvaniaNo Drawing. Application January 22, 1936,  
Serial No. 69,855

7 Claims. (Cl. 87-9)

This invention relates to the manufacture of lubricating compositions and it comprises improved methods of making compounded lubricants useful in lubricating metal surfaces either under ordinary or high pressure, particularly the latter, wherein oils of the sperm group, including sperm oil itself, and similar type oils are first sulfurized and then the sulfurized oils so obtained are compounded with suitable lubricating oils in sufficient amount to give a compounded lubricant having the desired properties, and it also comprises the improved sulfurized oils and lubricants so obtained, the compounded lubricant being stable in storage and in use and being substantially non-corrosive to metals; all as more fully hereinafter set forth and as claimed.

This application is in part a continuation of my prior copending application Serial No. 20 715,551, filed March 14, 1934, now United States Patent No. 2,065,247, patented December 22, 1936.

Mixtures of mineral oil with sulfurized oils are well known, such mixtures having been used as cutting oils, etc. Sulfurized fatty oils, obtained by adding sulfur to a fatty oil such as lard oil, etc., and heating the mixture for several hours have been frequently used in making such cutting oils. Likewise, it is well known that the addition of sulfurized oil to mineral oils imparts extreme pressure characteristics to them. There is a demand for lubricants which in the form of thin films are capable of withstanding high pressures, such as occur in the gears and transmissions of heavy duty motor trucks and high speed automobiles.

I have found that stable non-corrosive lubricants having the requisite commercial properties can be obtained by compounding minor amounts of sulfurized sperm oil with the usual mineral lubricating oils. In this way, I obtain superior compounded lubricants. By varying the amount of sulfurized sperm oil and the particular mineral oil used, a wide range of commercial lubricants can be obtained.

Although sperm oil is frequently termed a fatty oil, it is quite different from the ordinary fatty oils, which are tri-esters of glycerine. Sperm oil is composed principally of the fatty esters of monohydric alcohols of relatively high molecular weight; it being a mono-ester. Actually sperm oil is a liquid wax of the ester type. Being an ester, it is also different from the paraffin hydrocarbons commercially known as waxes.

Sperm oil is obtained from the head cavities and blubber of the cachetot or sperm whale (*Physeter macrocephalus*). The crude oil contains varying amounts of spermaceti and like solid waxes of the ester type. In refining the

oil, these waxes are removed by refrigeration and pressing, to obtain the commercial sperm oils. The commercial oils are known as winter sperm oil, spring sperm oil, etc., and are substantially free of solid waxes. The commercial 5 sperm oil is a thin yellow liquid and when of good quality is nearly free from odor. In the present invention it is advantageous to use refined sperm oil of good quality.

Sperm oil itself is a good lubricant. Being 10 both limpid and substantially free from any tendency to "gum" (usually resistant to oxidation and resinification), it has been long used to lubricate light machinery. Also, it has been blended with mineral oil to form compounded 15 lubricants. I have found that sulfurized sperm oil has enhanced lubricating qualities and has desirable viscosity and blending properties, making it exceedingly useful in compounding lubricants.

Generally, the lubricating compositions of the present invention comprise a major proportion of lubricating oil and a minor amount of a sulfurized sperm oil. Such lubricating compositions are particularly useful as extreme pressure lubricants. That is, they are satisfactory 25 for lubricating parts which are subjected to relatively high pressures. They have other advantageous properties arising from the inherent characteristics of the sulfurized sperm oil.

I have found that especially good results may be obtained by employing in the present invention, sulfurized sperm oils which have the following properties:

|                                      |           |    |
|--------------------------------------|-----------|----|
| Gravity, A. P. I.                    | 13.6-14.6 | 35 |
| Viscosity, S. U. V., 210° F. seconds | 200-300   |    |
| Pour: °F. (not greater than)         | +45       |    |
| Sulfur, per cent                     | 8-14      |    |
| Neutralization number                | 1-1.5     | 40 |

Sulfurized sperm oils having the above properties are readily soluble in all of the ordinary grades of lubricating oils. They are fully miscible and compatible with the high gravity oils, such as paraffinic base oils (Pennsylvania, etc.) 45 and solvent refined oils, etc., over a wide range of conditions such as temperature, proportions, etc. When they are compounded with such mineral oils, improved compounded lubricants are obtained which are remarkably stable, as well 50 as having viscosities, viscosity indexes, specific gravities, pour points, etc. capable of meeting the technical specifications for high grade commercial lubricants. Their lubricating qualities 55 over a wide range of utilization are excellent.

To produce such high grade sulfurized oils I find it is advantageous to use, as the starting material, commercial sperm oil having the

|                                                                  |             |
|------------------------------------------------------------------|-------------|
| following properties, for example, but not by way of limitation: |             |
| Specific gravity, 60°/60° F.                                     | 0.878-0.884 |
| Viscosity, S. U. V., 100° F.                                     | 95-110      |
| 5 Flash, O. C., minimum                                          | 490         |
| Pour, °F., maximum                                               | +40         |
| Color, N. P. A., not darker than                                 | 1.5         |
| Neutralization number, maximum                                   | 0.5         |
| 10 Oleic acid eq., per cent., maximum                            | 0.25        |
| Saponification number                                            | 125-135     |
| Iodine number                                                    | 80-90       |

The sulfur employed should be of good quality and free of any abrasive material such as sand, fossil fragments, etc. Sublimed sulfur, such as flowers of sulfur, is advantageous. However, any finely ground sulfur, such as sulfur flour, may be used.

The amount of sulfur used to sulfurize the sperm oil may be varied according to the particular sperm oil being processed and the specific characteristics desired in the final product. Usually the ratio of sulfur to oil is between 5:95 and 20:80. Generally, I employ substantially an amount of 25 sulfur not exceeding that necessary to saturate the double bonds of the sperm oil used. In controlling the ratio of sulfur to oil, some unsulfurized sperm oil may be present in the final product. This is permissible as unsulfurized sperm oil is 30 more or less a desirable and advantageous ingredient in certain lubricating compositions.

By properly controlling the sulfurizing operation, for instance, by employing the methods given post, the percentage of combined sulfur 35 in the sulfurized sperm oil is approximately that in the reaction mixture. Likewise, very little hydrogen sulfide is formed when the reaction is properly controlled.

In preparing the sulfurized sperm oil, the sperm 40 oil is reacted with suitable amounts of sulfur at temperatures between about 300-385° F., the reaction being continued until the sulfur is combined in the form of neutral organic sulfur compounds. However, to obtain superior sulfurized 45 sperm oils, I find it advantageous to use reaction temperatures between 335° and 360° F. and to employ controlled methods of sulfurization, wherein decomposition of the oil, side reactions, over-vulcanization, etc., are substantially avoided. 50 If the sulfurization is properly conducted, the viscosity of the oil sharply increases and then the viscosity tends to become substantially constant during the remainder of the heating.

In general, control of the sulfurization is obtained by first preheating the sperm oil to about 55 the lower reaction temperature (325° F.) or slightly below, and then gradually adding the required amount of sulfur to the preheated oil, the rate of addition being adjusted so that heat developed 60 during the addition of the sulfur gradually and quietly raises the reaction mixture to a temperature just below the preferred upper limit (360° F.). Advantageously, the finely divided sulfur may be gradually sifted into the oil while agitating. After all the sulfur has been added, the 65 temperature tends to drop slightly and then the reaction mixture is maintained at about 345° F. until the reaction is complete. The course of the reaction may be easily followed by withdrawing 70 test samples and determining the change in viscosity. After the proper viscosity has been obtained, the end point can easily be determined by diluting the sulfurized oil with a standard amount of mineral oil and determining its corrosive action upon a copper strip. When the cop-

per strip remains unattacked or shows only a slight stain, the reaction is complete. Then the sulfurized oil is cooled to about room temperature. It can be stored in metal drums or other suitable containers.

The copper strip test here employed was devised by me in 1917 for determining the relative corrosiveness of lubricating oils. The procedure is as follows:

A mechanically polished copper strip  $\frac{1}{2}$  inch 10 by 3 inches is immersed in 25 cc. of lubricant contained in a test tube which is placed in a boiling water bath and held at the temperature of boiling water for three hours. At the end of this time the strip is removed and adhering oil washed 15 off with a light naphtha and examined for evidence of corrosion. A negative test is one in which the strip shows only a slight stain or discoloration. The positive test is one where the strip shows considerable discoloration or tendency to scale, indicating presence of corrosive constituents in the lubricant.

In preparing the diluted sample for a test, I ordinarily use a standard mineral oil having the following properties:

|                              |          |
|------------------------------|----------|
| Gravity, A. P. I.            | 27.1     |
| Specific gravity, 60°/60° F. | 0.8922   |
| Viscosity, S. U. V.:         |          |
| 100° F.                      | 1059     |
| 130° F.                      | 420      |
| 210° F.                      | 89       |
| Viscosity index              | 92       |
| Flash, O. C., °F.            | 470      |
| Fire, O. C., °F.             | 545      |
| Pour, °F.                    | +5       |
| Color, N. P. A.              | dl. 4.25 |
| Carbon residue, percent      | 0.44     |
| Neutralization number        | 0.01     |

The sample of sulfurized sperm oil is diluted with 40 the above mineral oil in the ratio of 10:90 to obtain the sample used in determining the corrosion by the copper strip method. The copper strip is removed from the heated oil sample after 3 hours, and then wiped dry and inspected in the usual 45 manner. Sometimes, a test mixture the same as the desired compounded lubricant is used in the above test.

With the above mentioned controlled methods of sulfurization, there is but little loss of sulfur; 50 the percentage of combined sulfur in the sulfurized sperm oil is approximately that in the reaction mixture. During the sulfurization, very little hydrogen sulfide is formed. As the finely divided sulfur is gradually added to the hot oil 55 by sifting, etc., there may be more or less mechanical loss of sulfur. With careful operation, however, this loss may be minimized, if not entirely avoided.

The viscosity of the oil increases rather rapidly 60 as the sulfur is added and upon combination of most of the sulfur the viscosity tends to remain substantially constant as the heating is continued. Undesirably low reaction temperatures should be avoided for the best combination of the sulfur 65 and exceedingly high temperature should be avoided to prevent undesirable side reactions. By way of specific example as to the heating, with the sperm oil preheated to between 325-340° F. and the sulfur gradually added so as to bring 70 the reaction temperature to between 330 and 360° F., the maximum viscosity is obtained with 6 to 11 hours heating; all the sulfur being added during the first two hours. Upon maintaining the temperature at  $340 \pm 5$ ° F., all the sulfur can be 75

brought into combination in the form of neutral sulfur compounds within 16 to 24 hours, with but a slight decrease in the viscosity during digestion. Thus by following the reaction by means of viscosity tests upon test samples withdrawn from the batch and by means of corrosion test made at about the end point, satisfactory sulfurized sperm oil may be readily and consistently produced by my improved method; the details of ratios of sulfur to oil, of rate of addition of sulfur and of time of heating being adjusted to the particular materials and equipment used in commercial practice.

From the description ante, the ranges of temperature generally used are between 325 and 360° F. and the time of heating is between 16 and 24 hours, the sulfur being added during the first two hours. After the reaction is completed, the sulfurized oil is cooled to room temperature and, if desired, may be filtered or screened to remove any foreign bodies or abrasive materials that may have been accidentally introduced into the batch. As the sulfurized sperm oil is quite viscous, the filtration may be made while the oil is still hot. Sometimes the sulfurized oil may be centrifuged, but ordinarily this is unnecessary when care has been used to exclude introduction of foreign matter. However, centrifuging can be advantageously used in later stages of the processing as shown post.

The controlled method of sulfurization here employed has several advantages. By first pre-heating the sperm oil, it is more or less dried during that step; the water and other volatiles being evaporated. Removal of these volatiles helps to minimize side reactions and the production of corrosive sulfur compounds. Further, the sulfur more readily dissolves in the hot oil and a uniform mixture of the reactants is quickly and readily obtained. Stratification of a heavy layer of molten sulfur and oil, frequently encountered in sulfurizing fatty oils, can be entirely avoided by the present methods. The sulfur being added in finely divided form to the so-heated oil becomes converted into molten drops which completely dissolve in the oil before they have time to settle to the bottom of the reaction vessel. As the mixing is performed at reaction temperature, combination of the sulfur with the oil in the desired manner is immediately initiated and thus a high yield of neutral sulfur compounds is obtained. Likewise, the time of reaction is held to a minimum and decomposition of the oil and of the neutral sulfur compounds is avoided. Again, the elevated temperature used throughout the operation renders the sulfurized oil, as formed, more mobile thus facilitating the addition and mixing of the last portions of the sulfur. In accomplishing this result, the heat of reaction is permitted to increase slightly the temperature of the reaction mixture in the first stages. In turn, many of these advantageous results may be attributed to the gradual addition of the sulfur in the manner set forth ante. In this controlled method there is a worthwhile overall efficiency leading to a high yield of desirable sulfurized sperm oil of high purity with a minimum loss of materials.

The sulfurized sperm oil here obtained when added to mineral oil in minor amounts yields improved compounded lubricants. It may be advantageously compounded with any of the ordinary mineral lubricating oils to modify the properties thereof. Varying amounts of sulfurized sperm oil may be employed according to the com-

pounded lubricant desired and the mineral oil base used. By blending from one-tenth per cent to thirty per cent by weight of sulfurized sperm oil with the various types of lubricating oils and greases, I obtain a wide range of commercial lubricants wherein one or more properties of the lubricant are advantageously improved. Numerous illustrative embodiments of such commercial blended lubricants are given post. To form such blends or mixtures, various methods may be employed.

In making compound lubricants, the desired amount of sulfurized sperm oil is added to the selected mineral oil and the mixture heated and agitated until a uniform blend is obtained. By using temperatures between 70° and 200° F. for oils, and often higher temperatures for greases for this mixing, the sulfurized oil quickly blends with the oil or grease. Sometimes the oil or grease may be preheated to such temperatures before adding the sulfurized oil. Again the sulfurized oil while hot, for instance hot oil from the sulfurizing operation, may be run into unheated or preheated mineral oil. However, the mixing may be effected at room temperature; it being sometimes advantageous to dilute first the sulfurized oil with part of the mineral oil, forming, so to speak, a master batch of the extreme pressure ingredient and the mineral oil. Such master batch can be prepared hot, cooled, and then mixed in the bulk of the mineral oil in the cold. In any event, thorough agitation is employed to insure the production of uniform compounded lubricants. Suitable mechanical agitating devices may be used. Or a current of gas may be blown through the mixture to stir it. The gas in passing through the oil will remove any volatile compounds that may be dissolved therein. A current of air may be used for this purpose, but other gases, such as carbon dioxide, nitrogen, etc., may be employed. If high temperatures are used during the mixing and blending, the gas employed should be inert under the given conditions. Generally when the mixture is stirred and agitated by means of a current of air, etc., the desired blending is readily effected at room or slightly elevated temperature. For instance, 12 parts of sulfurized sperm oil and 88 parts of mineral oil may be easily blended by warming the mixture to about 160° F. and blowing a current of air through the warmed oil for about 60 minutes. The air will remove any trace of H<sub>2</sub>S that might have remained dissolved in the sulfurized oil. Blends or compound lubricants using other proportions of sulfurized and mineral oil may likewise be readily obtained by the above methods. The compound lubricant may be filtered or centrifuged, if desired.

In this way, valuable commercial lubricants useful for lubricating the differential and transmission units of automobiles may be produced; either a lubricant of winter or summer grade. The two grades can be easily obtained by simply varying the mineral oil base employed; it being only necessary to select a standard grade of winter or summer mineral oil and add the amount of sulfurized oil required to impart the desired extreme pressure characteristics thereto. Usually the sulfurized sperm oil and mineral oil are blended in ratios, by volume, between 10:90 and 14:86. The extreme pressure lubricants so produced are high-grade, stable non-corrosive materials. They show more than a 100 per cent increase in load carrying capacity over the base oil, as determined by either the Almen or Timken.

tests for E. P. lubricants. Being stable they can also be used for ordinary lubrication wherein the usual pressures are encountered.

The following examples are illustrative embodiments of the methods and products broadly set forth ante, and are not limitative of the invention.

*Example 1.*—This example illustrates an advantageous method of making the sulfurized sperm oil. A sperm oil having the following properties,

|                              |        |
|------------------------------|--------|
| Gravity, °A. P. I.           | 29.0   |
| Specific gravity, 60°/60° F. | 0.8816 |
| Viscosity, S. U. V.:         |        |
| 70° F.                       | 171    |
| 100° F.                      | 100    |
| 130° F.                      | 71     |
| 210° F.                      | 43.3   |
| Flash, O. C., °F.            | 505    |
| Pour, °F.                    | +35    |
| Color, Saybolt               | —5     |
| Neutralization number        | 0.14   |
| Saponification number        | 130.9  |
| Iodine number                | 87     |

was sulfurized under controlled conditions, using approximately 12 per cent sulfur by weight on the oil.

Into a direct-fired, 20-barrel, open-top grease kettle I charged 8057 lbs. of said sperm oil (1097 gal.) and gradually heated the oil to 320° F. in about 4 hours, while stirring. While continuing the stirring, 1098 lbs. of sulfur flour (approximately 1 lb. of sulfur per gallon of oil) was gradually added by sifting it into the hot oil over a period of two hours and at such a rate as to maintain a steady increase in temperature to 360° F. Then the temperature was gradually lowered to 340° F. and the reaction mixture maintained at that temperature and stirred for 16 hours; the heating then being stopped and the sulfurized oil cooled to normal temperature. The total time from the first addition of sulfur to the completion of the reaction was about 20 hours.

In the above type operation, after the reaction has been initiated, the fire may be drawn or cut off during the addition of the rest of the sulfur, but usually it is only lowered so as to prevent undue loss of heat by radiation. After the reaction mixture is brought to 340° F., the fire is increased to hold that temperature during the remainder of the reaction. The change in viscosity during the reaction was as follows:

|    | After first addition of sulfur, hours | Viscosity, S. U. V. at 210° F., seconds |
|----|---------------------------------------|-----------------------------------------|
| 1  |                                       | 68                                      |
| 2  |                                       | 177                                     |
| 4  |                                       | 287                                     |
| 8  |                                       | 276                                     |
| 12 |                                       | 268                                     |
| 16 |                                       | 242                                     |

Operating in this way, there was obtained 9064 lbs. of sulfurized oil; the percentage yield by weight being 99.0 per cent of the materials charged. As part of the loss is due to evaporated water and other volatiles from the sperm oil and sulfur, clearly only a very small amount of H<sub>2</sub>S is formed. During the sulfurization a slight odor of hydrogen sulfide was detectable, but the sulfurized oil did not have an objectionable odor. During sulfurization the oil increased in volume and the yield by volume was 1120 gallons. The

sulfurized oil so obtained was of high quality and had the following properties:

|                              |        |
|------------------------------|--------|
| Gravity, °A. P. I.           | 14.1   |
| Specific gravity, 60°/60° F. | 0.9718 |
| Pounds per gallon            | 8.093  |
| Viscosity, S. U. V., 210° F. | 242    |
| Pour, °F.                    | +45    |
| Sulfur (B) : per cent        | 11.10  |
| Neutralization number        | 0.63   |
| Color, N. P. A.              | Dark   |

It is readily soluble or dispersible in mineral oil of various grades. When diluted with 90 parts of mineral oil to 10 parts of sulfurized oil, the diluted oil gave only a slight tarnish by the copper strip test.

*Example 2.*—This example illustrates the manufacture of extreme pressure lubricants from these sulfurized sperm oils and suitable mineral oil bases. A mineral oil (winter grade) was employed, which had the following properties:

|                              |        |
|------------------------------|--------|
| Gravity, °A. P. I.           | 27.1   |
| Specific gravity, 60°/60° F. | 0.8922 |
| Viscosity, S. U. V.:         |        |
| 100° F.                      | 1059   |
| 130° F.                      | 420    |
| 210° F.                      | 89     |
| Viscosity index              | 92     |
| Flash, O. C., °F.            | 470    |
| Fire, O. C., °F.             | 545    |
| Pour, °F.                    | +5     |
| Color, N. P. A.              | dil    |
| Carbon residue, per cent     | 0.44   |
| Neutralization number        | 0.01   |

To 88 gallons of the above mineral oil, there was added 12 gallons of the sulfurized sperm oil obtained in Example 1. The mixture was warmed to 160° F. and a current of air blown through it, until a uniform blend was obtained. This required about one hour. The product was filtered, but no significant amount of foreign matter was found to be present.

The compound lubricant so obtained is an excellent winter grade E. P. lubricant and has the following properties:

|                                  |                |
|----------------------------------|----------------|
| Gravity, °A. P. I.               | 25.4           |
| Specific gravity, 60°/60° F.     | 0.9018         |
| Viscosity, S. U. V.:             |                |
| 100° F.                          | 1144           |
| 130° F.                          | 469            |
| 210° F.                          | 98             |
| Viscosity, furol, 100° F.        | 116            |
| Viscosity index                  | 100            |
| Flash, O. C., °F.                | 480            |
| Fire, O. C., °F.                 | 555            |
| Pour, °F.                        | 0              |
| Color, N. P. A.                  | dil            |
| Sulfur, per cent                 | 5.5            |
| Carbon residue, per cent         | 1.48           |
| Precipitation number             | 0.52           |
| Neutralization number            | 0.08           |
| Corrosion test, 212° F., 3 hours | Slight tarnish |
| Steel strips, 212° F., 24 hours: |                |

|                            |     |
|----------------------------|-----|
| Dry lubricant—             |     |
| Tarnish                    | Nil |
| Loss, mg                   | 0.2 |
| Wet lubricant (10% water)— |     |
| Tarnish                    | Nil |
| Loss, mg                   | 0.1 |

|                                                               |       |
|---------------------------------------------------------------|-------|
| Ash, per cent                                                 | 0.002 |
| Centrifuge test: 2 hours room temperature, per cent separated | Trace |

To obtain a summer grade extreme pressure lubricant by the above procedure, in lieu of the

winter grade mineral oil, there is substituted a summer grade oil having the following properties:

|    |                                                                  |                |     |  |  |  |
|----|------------------------------------------------------------------|----------------|-----|--|--|--|
| 5  | Gravity, °A. P. I.                                               | 25.1           |     |  |  |  |
| 5  | Specific gravity, 60°/60° F.                                     | 0.9038         |     |  |  |  |
| 5  | Viscosity, S. U. V.:                                             |                |     |  |  |  |
| 10 | 100° F.                                                          | 4329           |     |  |  |  |
| 10 | 130° F.                                                          | 1513           |     |  |  |  |
| 10 | 210° F.                                                          | 206            |     |  |  |  |
| 10 | Viscosity index                                                  | 94             |     |  |  |  |
| 10 | Flash, O. C., °F.                                                | 580            |     |  |  |  |
| 10 | Fire, O. C., °F.                                                 | 670            |     |  |  |  |
| 10 | Pour, °F.                                                        | +5             |     |  |  |  |
| 10 | Color, N. P. A.                                                  | dil            | 7.0 |  |  |  |
| 15 | Carbon residue, per cent                                         | 1.30           |     |  |  |  |
| 15 | Neutralization number                                            | 0.01           |     |  |  |  |
| 20 | The compound lubricant so obtained has the following properties: |                |     |  |  |  |
| 20 | Gravity, °A. P. I.                                               | 23.6           |     |  |  |  |
| 20 | Specific gravity, 60°/60° F.                                     | 0.9123         |     |  |  |  |
| 20 | Viscosity, S. U. V.:                                             |                |     |  |  |  |
| 20 | 100° F.                                                          | 3738           |     |  |  |  |
| 20 | 130° F.                                                          | 1324           |     |  |  |  |
| 20 | 210° F.                                                          | 203            |     |  |  |  |
| 20 | Viscosity, furol, 100° F.                                        | 379            |     |  |  |  |
| 20 | Viscosity index                                                  | 101            |     |  |  |  |
| 20 | Flash, O. C., °F.                                                | 585            |     |  |  |  |
| 20 | Fire, O. C., °F.                                                 | 650            |     |  |  |  |
| 20 | Pour, °F.                                                        | +5             |     |  |  |  |
| 20 | Color, N. P. A.                                                  | dil            | 8.0 |  |  |  |
| 20 | Sulfur, per cent                                                 | 1.56           |     |  |  |  |
| 20 | Carbon residue, per cent                                         | 1.36           |     |  |  |  |
| 20 | Precipitation number                                             | 0.03           |     |  |  |  |
| 35 | Neutralization number                                            | 0.09           |     |  |  |  |
| 35 | Corrosion test, 212° F., 3 hours                                 | Slight tarnish |     |  |  |  |
| 35 | Steel strips, 212° F., 24 hours:                                 |                |     |  |  |  |
| 35 | Dry lubricant—                                                   |                |     |  |  |  |
| 35 | Tarnish                                                          | Nil            |     |  |  |  |
| 40 | Loss, mg.                                                        | 0.1            |     |  |  |  |
| 40 | Wet lubricant (10% water)—                                       |                |     |  |  |  |
| 40 | Tarnish                                                          | Nil            |     |  |  |  |
| 40 | Loss, mg.                                                        | 0.1            |     |  |  |  |
| 40 | Ash, per cent                                                    | 0.004          |     |  |  |  |
| 45 | Centrifuge test, 2 hours room temperature, per cent separated    | Trace          |     |  |  |  |

From the properties of the mineral oils and of the extreme pressure lubricants, given ante, it is clear that the added sulfurized sperm oil does not deleteriously alter the desirable physical properties of the mineral oil, such as viscosity, pour point, etc., although it does impart good extreme pressure characteristics thereto. The improvement in the extreme pressure characteristics obtained is shown by the results of tests made upon the products of Example 2, which are as follows; an average mineral oil being included for purposes of comparison:

|    | Test conditions           | Winter grade | Summer grade | Average mineral oil % |     |
|----|---------------------------|--------------|--------------|-----------------------|-----|
| 60 |                           |              |              |                       |     |
| 65 | Almen test:               |              |              |                       |     |
| 65 | Journal speed, R. P. M.   | 600          | 600          | 600                   | 600 |
| 65 | Rubbing speed, ft./min.   | 40           | 40           | 40                    | 40  |
| 65 | Lever load, pounds        | 20           | 18           | 18                    | 8   |
| 65 | Torque, pounds ft./10     | 19           | 19           | 19                    | 15  |
| 65 | Unit load, lb./sq. in.    | 10,000       | 9,000        | 4,000                 |     |
| 70 | Timken test:              |              |              |                       |     |
| 70 | Duration of test, minutes | 10           | 10           | 10                    | 10  |
| 70 | Journal speed, R. P. M.   | 200          | 800          | 800                   | 800 |
| 70 | Rubbing speed, ft./min.   | 400          | 400          | 400                   | 400 |
| 70 | Lever load, pounds        | 42           | 42           | 42                    | 7   |
| 70 | Unit load, lb./sq. in.    | 18,600       | 22,200       | 7,000                 |     |
| 70 | Scar width, inches        | 0.0460       | 0.0377       | 0.020                 |     |
| 70 | Metal loss, milligrams    | 1.3          | 1.5          | 0.5                   |     |

75 ° Without added sulfurized oil.

In the above examples, the ratios and other details may be varied as indicated in the general description ante, to obtain various specific products. Two or more mineral oils may be mixed and blended to obtain suitable or special mineral bases for making the E. P. lubricant, if necessary or desirable.

By the various methods shown, I obtain a series of compound lubricants having properties meeting the following specifications for superior E. P. lubricants:

|                                                                             | General              | Winter grade | Summer grade |    |
|-----------------------------------------------------------------------------|----------------------|--------------|--------------|----|
| Gravity, °A. P. I.                                                          | 23.0-23.5            | 24.5-25.5    | 23.0-25.0    | 15 |
| Viscosity, S. U. V., 210° F.                                                | 95-210               | 95-100       | 200-210      |    |
| Flash, O. C., °F. (min.)                                                    | 460                  | 460          | 560          |    |
| Pour, °F.                                                                   | +5 to +15            | +5           | +15          |    |
| Sulfur, percent (max.)                                                      | 1.40                 | 1.49         | 1.40         |    |
| Corrosion test, 212° F., 3 hours                                            | Slight tarnish only. | Same         | Same         |    |
| Centrifuge test, 2 hours room temperature, percent separated (max.)         | 0.05                 | 0.05         | 0.05         | 20 |
| Load capacity:                                                              |                      |              |              |    |
| Almen rating, 600 R. P. M., lever load, pounds (min.)                       | 16                   | 16           | 16           | 25 |
| Timken rating, 800 R. P. M.—10°-135° F., 10 min., lever load, pounds (min.) | 40                   | 40           | 40           |    |

In producing such E. P. lubricants, generally I find it is advantageous to use sulfurized sperm oils having the following properties:

|                                                                                                                                                      |           |
|------------------------------------------------------------------------------------------------------------------------------------------------------|-----------|
| Viscosity, S. U. V. 210° F.                                                                                                                          | 200-300   |
| Sulfur, per cent                                                                                                                                     | 10.0-12.0 |
| and compound them with a suitable mineral oil base; 12 volumes of such sulfurized oil to 88 volumes of mineral oil base being an advantageous ratio. | 35        |

The examples of mineral oil bases used are for purposes of illustration. Naphthenic oils, oils of mixed bases, and in fact any commercial oil may be used.

The sulfurized sperm oils made by the present methods may be used in making the pipe thread lubricants disclosed in my copending application Ser. No. 60,356 to obtain improved products by the methods there shown. Likewise, the E. P. lubricating oils of the present invention may be further compounded with other ingredients such as soaps, graphite, finely divided metals, bodied vegetable, animal and fish oil, etc., to obtain special products such as greases and the like.

A decided advantage of sulfurized sperm oil in a lubricant is that under normal lubricating conditions it is better than the usual oil, and its presence in a lubricating composition makes it particularly useful when extreme pressure lubricants are needed.

The compound lubricants exemplified by Example 2 have a number of advantages that are not readily apparent from the usual inspection of this type of compounds. For example, the sulfurized sperm oil is very soluble and compatible with the higher gravity oils over a wide range of temperatures and proportions. Furthermore, these sulfurized sperm oils permit the use of high gravity oils, which results in a compound lubricant that is very resistant to changes in viscosity under the more severe uses. Such lubricants, in addition to resisting viscosity changes, resist the usual tendency of certain types of compound lubricants to "string" or separate in use.

As an example of the stability and utility of compound lubricants as exemplified in Example 2, a heavy duty worm driven truck differential was charged with this lubricant and operated

continuously for nine months, covering during this period a total of 60,000 miles, the majority of the time under very heavy loads. During this period the lubricant increased in viscosity only 5 8 seconds at 210° F., S. U. V.; while a sulfurized compound lubricant containing one of the usual sulfurized fatty oils was completely solidified in a similar test after 20,000 miles. The solubility of the sulfurized sperm oil was unaffected by this 10 severe test and the lubricant showed no evidence of stratification or segregation of constituents as shown by the centrifuge test.

The compounded oils utilizing the sulfurized sperm oil as described are particularly useful in 13 a number of relations, as, for instance, marine engine oils, motor oils and in making locomotive driving journal compounds where special greases are needed.

In steam cylinder lubricants where relatively 20 high temperatures and rubbing speeds prevail, my compound has decided advantages over the usual rape seed oil bodied compounds. Such compounds containing rape seed oil and naphthenic or coastal type of lubricating oils can be 25 advantageously improved and made particularly useful for marine engine oils by the addition of a few per cent of a sulfurized sperm oil, say 3 to 5 per cent. In such a compound the contained sperm oil increases the oiliness and assists the 30 dispersion of the bodied rape seed oil, whereby the compound retains its lubricating qualities in the upper limits of permissible temperatures and rubbing speeds.

With the present tendency of automobile 35 manufacturers to use special bearing alloys, such as cadmium-silver alloys, cadmium-nickel alloys, copper-lead alloys, and the like, there is a demand for certain grades of lubricants which will not have corrosive action on them. I have found 40 that a small percentage (0.1 to 1.0 per cent) of sulfurized sperm oil in motor oils having high viscosity index, such as Pennsylvania base oils and solvent refined oils, will eliminate the corrosive action on the special type of alloy bearings 45 to which reference has been made.

In greases used for locomotive driving journals and the like the melting point must necessarily be rather high, with the result that the wetting power of the lubricating constituent is 50 somewhat limited. The addition of sulfurized sperm oil to such compound imparts a decided "oiliness" or wetting power, even when as low as 1 to 2 per cent is used in greases of this type.

In types of greases such as those used in automobile wheel bearings, high speed ball bearings and the like, where the lubricants function under relatively mild bearing loads but high bearing speeds, from 2 to 10 per cent of sulfurized sperm oil can be used to decided advantage.

60 A typical good marine engine oil comprising sulfurized sperm oil is shown in the following example:

Example 3.—In preparing a marine engine oil I employ the following oil:

|                          |      |
|--------------------------|------|
| Gravity, "A. P. I.       | 20.6 |
| Viscosity, S. U. V.:     |      |
| 100° F.                  | 1268 |
| 210° F.                  | 75   |
| 70 Flash, O. C., °F.     | 430  |
| Fire, O. C., °F.         | 490  |
| Pour, °F.                | —5   |
| Color, N. P. A.          | 4.75 |
| Carbon residue, percent  | 0.20 |
| 75 Neutralization number | 0.02 |

and to 70 parts of such oil, I add 5 parts of sulfurized sperm oil and 25 parts of blown rape seed oil.

Example 4.—In preparing a marine engine oil I employ the following coastal lubricating oil distillate of the following properties:

|                         |        |
|-------------------------|--------|
| Gravity, "A. P. I.      | 20.7   |
| Viscosity, S. U. V.:    |        |
| 100° F.                 | 1886   |
| 210° F.                 | 89 10  |
| Flash, O. C., °F.       | 470    |
| Fire, O. C., °F.        | 545    |
| Pour, °F.               | —5     |
| Color, N. P. A.         | 4.5    |
| Carbon residue, percent | 0.3 15 |
| Neutralization number   | 0.02   |

and to 70 parts such oil I add 3 parts of sulfurized sperm oil and 27 parts blown rapeseed oil.

The following is illustrative of a typical motor oil:

|                         |         |
|-------------------------|---------|
| Gravity, "A. P. I.      | 31.4    |
| Viscosity, S. U. V.:    |         |
| 100° F.                 | 369     |
| 210° F.                 | 60 25   |
| Flash, O. C., °F.       | 440     |
| Fire, O. C., °F.        | 505     |
| Pour, °F.               | —5      |
| Color, N. P. A.         | 2.5     |
| Carbon residue, percent | 0.13 30 |
| Neutralization number   | Nil     |

and to 100 parts of this oil, I add 0.75 part by weight of sulfurized sperm oil.

The following is an illustration of a locomotive driving journal compound:

|                                                       |         |
|-------------------------------------------------------|---------|
| Make-up, percent by weight:                           |         |
| 150 dark filtered cylinder stock                      | 42.9    |
| Sodium-stearic acid soap                              | 3.0     |
| Sodium-tallow oil soap                                | 49.5 40 |
| Sulfurized sperm oil                                  | 4.6     |
| Oil of cassia                                         | 0.003   |
| Inspection penetration, A. S. T. M., 77° F., unworked | 66      |

The following is a typically good steam cylinder lubricant:

|                                             |               |
|---------------------------------------------|---------------|
| Make-up, percent by volume:                 |               |
| 120 vis./210° F. Mid-Continent Bright stock | percent 30 50 |
| 150 vis./210° F. Mid-Continent Bright stock | percent 10    |
| Sulfurized sperm oil                        | do 5          |
| Acidless tallow                             | do 5          |
| Inspection:                                 | 55            |

|                              |      |
|------------------------------|------|
| Gravity, "A. P. I.           | 26.1 |
| Viscosity, S. U. V., 210° F. | 115  |
| Flash, O. C., °F.            | 510  |
| Pour, °F.                    | +15  |

The following is a typically good grease for automobile wheel bearings, high speed ball bearings and the like:

|                             |          |
|-----------------------------|----------|
| Make-up, percent by weight: |          |
| 300 red paraffine oil       | 79.5 65  |
| Sulfurized sperm oil        | 4.8      |
| Sodium tallow soap          | 13.9     |
| Glycerine                   | 1.4      |
| Water                       | 0.4      |
| Oil of cassia               | 0.002 70 |
| Inspection:                 |          |

|                                            |     |
|--------------------------------------------|-----|
| Melting point, °F. Hawkhurst               | 158 |
| Penetration A. S. T. M., 77° F., un-worked | 317 |

The addition of sulfurized sperm oil to lubri-

cating compositions has several advantages. Its presence in the lubricating compositions renders the lubricant useful as an extreme pressure lubricant wherever desired. Further, the sulfurized sperm oil also functions as a corrosion inhibitor and renders the composition generally more stable. In compositions containing other ingredients in addition to the mineral oil, the sulfurized sperm oil serves as a blending agent increasing the uniformity of the mixture. Likewise it is useful in increasing the oiliness of the compounded lubricants. In other words, the sulfurized sperm oil in the composition set forth ante has many and diverse effects and functions, all of which are advantageous.

As stated ante, in lieu of sperm oil itself (oil from the cachetot whale) other "oils" of the sperm oil group may be used in making the sulfurized products according to this invention. For instance, bottlenose oil (dogeeling oil) may be employed. It is obtained from several species of toothed cetaceans, particularly the bottlenose whale (*Hyperoodon rostratum*); hence the name "bottlenose oil". It is so like true sperm oil in character, that the commercial oil is known as arctic sperm oil. The said class of oils have certain properties in common with true sperm oil; all of these oils containing characteristic types of fatty esters.

As is well known, true sperm oil is a mixture of certain esters. Those esters are the esters of monohydric alcohols with fatty acids of the oleic series, such esters having the following general formula



wherein R represents an aliphatic chain of relatively high molecular weight; the acid component being likewise of high molecular weight. From the information available, such as reported analysis, the principal and characteristic components of sperm oil and similar oils of the sperm oil group are mono-esters which are unsaturated or contain double bonds, on each side of the ester group. That is, they are esters of oleic acid or homologous acids of the oleic type with monohydric alcohols of the ethylene series (the series of alcohols corresponding to the oleic series of acids). This characteristic class of mono-esters may be represented by the following formula,



wherein n is at least 1.

Commercial sperm oil contains minor amounts of other fatty esters but the above mentioned class of esters are the characteristic components thereof. Thus any oil and mixture of esters containing the said characteristic esters are useful in the present invention. Such esters when sulfurized to form neutral organic sulfur compounds may be advantageously employed in making the compound lubricants set forth ante. For the present purposes, esters of this class which have a relatively high molecular weight are advantageous. That is, the sub-class of esters having the following formula:



wherein x is 1 to 7, are advantageous for making the said neutral sulfurized product. In sulfurizing them by the present methods, the added sulfur saturates the double bonds of such esters yielding products having neutrally combined sulfur in each half of the ester. Taking the oleate of oleyl alcohol (oleyl ester of oleic acid) where in the x of the above formula is 5, as an illustration, the neutral product may be represented by the following formula:



In my copending application Serial No. 60,357, I have described and claimed the manufacture of improved lubricants wherein sulfurized esters of fatty acids are added in minor amount to lubricating compositions, in which the lubricating base is or contains a major amount of mineral oil. The present application is in part a continuation of the above mentioned application and is directed to an advantageous species of the said generic invention wherein the sulfurized products employed are obtained from sperm oil or the fatty esters characteristic thereof.

While in the foregoing examples I have described direct sulfurization of the sperm oil, I at times find it advantageous to sulfurize sperm oil in the presence of another oil, as for instance a petroleum hydrocarbon oil which may well be the same as the oil used for the base for manufacturing the compound lubricant. That is, some of the mineral oil is mixed with the sperm oil prior to the addition of the sulfur.

What I claim is:

1. As an improved compound lubricant, a uniform blend of a major amount of mineral oil lubricating base and a minor amount of sulfurized sperm oil, said lubricant being stable both in storage and in use and being non-corrosive to metals.

2. As an improved lubricant, a compound lubricant having the following properties:

|                                                                  |           |    |
|------------------------------------------------------------------|-----------|----|
| Gravity, A. P. I.                                                | 23.0-26.5 | 50 |
| Viscosity, S. U. V., 210° F.                                     | 95-210    |    |
| Flash, O. C., °F., minimum                                       | 460       |    |
| Pour, °F.                                                        | +5 to +15 |    |
| Sulfur, per cent, minimum                                        | 1.40      |    |
| Corrosion test, 212° F., 3 hours. Slight tarnish only            | 55        |    |
| Centrifuge test, 2 hrs., room temp., per cent separated, maximum | 0.05      |    |
| Load capacity:                                                   |           |    |

Abram rating—

600 R. P. M., lever load, lb., minimum

16

Timken rating—

800 R. P. M., 100° F.-135° F., 10 minutes, lever load, lb.,

40 65

minimum

said lubricant comprising a mineral lubricating oil and a small amount of a neutral organic sulfur compound dissolved therein, said organic sulfur compound being a sulfurized sperm oil.

3. The lubricant of claim 2 wherein said sulfurized sperm oil is a sulfurized sperm oil containing 10 to 14 per cent sulfur stably combined and having a viscosity at 210° F. of between 225 and 275 seconds.

4. As a composition of matter, useful as a lubricant, a stable non-corrosive uniform composition comprising a mineral oil and a substantially neutral organic sulfide having the following formula:

action but which would normally tend to corrode the aforesaid alloy, and maintaining the effectiveness of the lubricating oil by incorporating therein sulfurized sperm oil in a small but sufficient proportion to retard the corrosion.



wherein  $x$  is at least 1.

15 5. A method of lubricating bearing surfaces which comprises maintaining between the bearing surfaces, one of which is an alloy selected from the class of cadmium-silver, cadmium-nickel, and copper lead alloys, a film of lubricating oil which initially produces an effective lubricating

6. As a composition of matter, useful as a lubricant, a composition comprising a major proportion of mineral oil and a minor proportion of a stable organic sulfur compound, said organic sulfur compound being a sulfurized naturally occurring ester of a monohydric alcohol and a high molecular weight fatty acid.

7. An improved lubricant composition comprising a major amount of a mineral oil lubricating base and a minor amount, sufficient to improve the lubricating characteristics of said base under conditions of use, of sulfurized sperm oil. 13

**HERSCHEL G. SMITH.**